

Aug. 4, 1942.

G. M. CALHOUN

2,292,047

AMMUNITION

Filed March 18, 1939



GORDON M. CALHOUN

INVENTOR.

BY

*D. Werner Smythe*  
ATTORNEYS.

## UNITED STATES PATENT OFFICE

2,292,047

## AMMUNITION

Gordon M. Calhoun, Stratford, Conn., assignor to  
Remington Arms Company, Inc., a corporation  
of Delaware

Application March 18, 1939, Serial No. 262,594

6 Claims. (Cl. 102—26)

This invention relates to projectiles for small bore cartridges, and contemplates an economical and relatively harmless projectile for short range work so designed that upon impact its kinetic energy is dissipated in such a manner as to substantially obviate the danger of injury to adjacent objects.

There are now in quite general use shooting galleries and devices of relatively short range, ordinarily intended for the use of conventional .22 caliber cartridges. The actual shooting range, that is the distance from the muzzle of the rifle to the target, in some shooting apparatus does not exceed six feet and the target to be hit is proportionately small. The energy of any of the ordinary .22 caliber cartridges, even those identified as "CB" or "BB" caps, is unnecessarily great for these ranges, and such excess energy is undesirable since it must be dissipated in some way upon the impact of the bullet. Solid lead bullets, and even such disintegrating lead bullets as described in the patent to Woodford, No. 2,168,381, August 8, 1939, are undesirable at these extremely short ranges, since their impact inevitably results in a shower of metallic fragments. Some of these fragments are inevitably of appreciable size, and even the enclosing of the entire apparatus in a cabinet provided only with an opening of sufficient size to permit manipulation of the gun has been found not wholly effective in the preventing of personal injuries.

In the drawing:

Fig. 1 is a sectional view of a projectile and shell employing my invention.

Fig. 2 is a modification of the use of my invention.

The present invention contemplates a bullet or projectile which is preferably entirely non-metallic, although metals in a fine state of division may be utilized. The bullet is of relatively light weight, but sufficiently rugged to withstand the stresses incident to firing, and sufficiently accurate for ranges of several times the range of the type of apparatus above-mentioned. It has been found that excellent projectiles for this purpose may be made from an admixture of a granular metallic oxide or salt with a binder. Preferably the binder is an admixture of a high melting microcrystalline petrolatum wax, such as "Socony 2300" and a high melting crystalline wax, such as "Shell Ceresin." In the fractional distillation of petroleum, various waxes are obtained. Paraffin wax is the crystalline wax recovered from the light lubricating oil fractions and may be obtained in various manners. The

5 heavy oil lubricating fraction that lies above the paraffin wax fraction or light lubricating oil distillate contains wax of a different characteristic than that of the paraffin fraction, the structure of this latter wax being amorphous or micro-crystalline. The wax in this higher viscosity distillate is sometimes referred to as "slop wax" and is not recoverable by the usual pressing or filtering method, which may be used for paraffin wax. There are various methods used to recover this wax which are well-known in the art, such as the "cold settling" method, or by the use of a solvent such as naphtha, for example. The petroleum residue left in the still after the higher viscosity distillates have been driven off may also have the wax therein recovered by a similar method such as the use of naphtha followed by a centrifuge or separation process. There are many other methods and solvents that might be used for the purpose of recovering the amorphous or microcrystalline waxes, all of which are familiar to those skilled in the art. Microcrystalline waxes apparently come from the residue after the paraffin wax fraction has been removed. "Petrolatum wax," when used in this specification, means a wax other than the paraffin waxes which are derived from the heavier distillates and residues. This wax has a higher melting point than the paraffin waxes of commerce, being as high as 180° F., and is a tough rubbery substance varying in color, in dependence upon the amount of refining to which it has been subjected. Petrolatum wax is to be understood not to mean petroleum jelly. "Shell Ceresin," supplied under that name by the Shell Union Oil Company, is a high melting crystalline, rather than microcrystalline, wax having a melting point of about 180° F. Any hard crystalline wax having a melting point between 175° and 190° F. 10 will perform satisfactorily. Excellent results have also been secured with a binder of the type commercially known as "Parakote," this being a composition comprising a high percentage of rubber of a relatively low vulcanization admixed with a relatively small percentage of a wax such as paraffin. The preferred filler material is litharge, although such other metallic oxides and salts as the oxides of iron and tungsten, iron sulphate, calcium tungstate, manganese tungstate, barium sulphate, barium carbonate, and the chromates, carbonates, sulphides and sulphates of lead may be used. In the event that greater density is desired for longer range work, powdered iron, lead or tungsten, may replace the metallic oxide or salt wholly or in part.

A preferred composition comprises about 80% of litharge, about 18% of a mixture of equal parts of "Socony 2300" and "Shell Ceresin," and about 2% of lamp black, the latter being added to produce a desired dark color and to serve as a filler.

It has also been found that some material such as powdered talc may be dusted on the projectile to make the bullet cleaner to handle.

The bullet composition is prepared by first melting the wax and stirring into the melted wax the desired quantity of a filler, such as litharge, and the desired amount of coloring matter, such as lamp black. After cooling, the cakes of material thus prepared may be stored for use when needed; at which time they are preferably somewhat softened by heat and forced through an extruding die into a wire, the wire being subsequently cut into sections from which bullets are swaged in the usual manner. In an alternative method of procedure, the cakes of the composition may be broken up, fragments softened by heat, if desired, and the softened material forced into bullet slug cavities of suitable size in a molding plate, there being a substantial number of such cavities in a single plate. Bullets are then swaged from the resulting slugs. Such bullets when loaded into cartridge shells containing priming and powder charges comparable with those used for .22 short lead bullet cartridges are reasonably accurate for ranges up to about 50 feet. Their accuracy at shorter ranges is increased by diminishing the powder charge; for extremely short range work, say ranges up to 10 feet, the most satisfactory results are secured with a very light propellant charge and a short bullet. To minimize the danger of injury to the relatively soft bullet, a cartridge shell of ordinary length, say .22 short, may be used, and a substantial fraction of the length of the bullet housed within the cartridge case.

In Fig. 1 is found an illustration of my invention in use in the conventional manner, 3 being the projectile and 4 the cartridge case. In Fig. 2 is found an example of my invention wherein I have put the projectile 5 within the cartridge shell 4 to minimize the danger of injury, 4 being the same as in Fig. 1.

It is to be understood that the invention extends to all equivalent compositions and procedures falling within a broad interpretation of the appended claims.

What is claimed is:

1. A projectile for small arms ammunition comprising a filler of a metallic oxide, and a binder of a high melting petroleum base wax.

2. A projectile for small arms ammunition comprising a filler of a granular metallic oxide held in a binder which is an admixture of high melting petroleum base waxes.

3. A projectile for small arms ammunition containing substantially 80 parts of litharge, and substantially 18 parts of a binder which is an admixture of high melting petroleum base waxes.

4. A projectile for small arms ammunition containing substantially 80% of litharge, 2% of lamp black, and 18% of a binder which is an admixture of high melting petroleum base waxes.

5. A projectile for small arms ammunition composed chiefly of a heavy finely divided granular metallic compound held in a binder which is an admixture of rubber and wax.

6. A projectile for small arms ammunition comprising a filler of heavy granular metallic compound held in a binder which is an admixture of a microcrystalline petrolatum wax having a melting point of between 120 and 175° F., and a crystalline wax having a melting point of between about 175 and 190° F.

GORDON M. CALHOUN.